

## UNITED STATES PATENT OFFICE

2,324,770

## LOW TEMPERATURE HYDRAULIC MEDIUM

Theodore E. Donlan, Union, N. J., assignor to  
Standard Oil Development Company, a cor-  
poration of Delaware

No Drawing. Application January 2, 1941,  
Serial No. 372,895

3 Claims. (Cl. 252—76)

This invention relates to liquid compositions suitable for use in fluid cooling and in fluid pressure transmitting systems. It relates particularly to anti-freeze compositions for the cooling systems of automobile engines.

It is well recognized that water is the most advantageous fluid cooling and fluid pressure transmitting medium at temperatures above its freezing point. The disadvantages, however, of its use at temperatures below its freezing point are such as to preclude its use in cooling systems and pressure transmitting devices which are likely to be operated at such low temperatures. Some improvement has been effected by dissolving in water substances which effect a lowering of the freezing point and which also effect a reduction of the relative degree of expansion upon solidification. The substances employed in these capacities are of two types, namely electrolytes, such as calcium chloride; and organic compounds miscible with water, of low freezing points and viscous consistencies at low temperatures such as the alcohols. Of these two types, the organic compounds are generally considered preferable because of the less corrosive nature of their aqueous solutions and the formation of viscous masses before solidification.

It has been found necessary to combat even this mild form of corrosion of the organic solutions when employed in the cooling system of internal combustion engines. The automobile cooling system consists essentially of three parts, the metal framework, the liquid heat transfer medium, and the mechanism for circulating the liquid in the metal framework. In the operation of the engine local overheating occurs, and due to the many and varied metal contacts in the metal framework and to air which may pass through the system as a result of the leakage of air through the pumping and packing equipment, corrosion occurs in many parts as a result of oxidation and development of electrochemical relations at the metallic surfaces. To repress this corrosion the compounds employed as inhibitors must be sensitive to the reactions involved especially as those with solder in view of its use as a jointing material. Furthermore, the solutions must be without effect upon rubber which is usually employed as a flexible connection between certain parts of the radiator system. The

compounds of this invention employed as inhibitors for fluid cooling and fluid pressure transmitting devices are effective in repressing the corrosion of all types of metallic surfaces likely to be encountered in the fabrication of automobile radiators, and they are also without effect on rubber.

An object of this invention is the preparation of compositions suitable for use in the cooling systems of automobile engines and other internal combustion engines, which are substantially non-corrosive to various metals in contact with one another in the automobile cooling system even when diluted with water in large quantities, and which do not readily deteriorate under service conditions or cause the deposition of gummy or resinous materials which impede the functioning of the cooling liquid.

Other objects of the invention will be apparent from the reading of the following description.

The compositions of the invention have, in addition to the usual constituents of hydraulic media suitable for use at low temperatures, small amounts of the phthalates of the metals above aluminum in the electromotive series of the elements. Among the phthalates which are particularly advantageous are those of the metals of sodium, potassium, barium, calcium and magnesium. It has been found that small quantities of these phthalates in the compositions are particularly effective as corrosion inhibitors for repressing the deterioration of the metallic surfaces and particularly the solder joints in the metal framework. Furthermore there is reason to believe that the phthalates contribute appreciably to the formation of an anti-corrosive film over the surface of the metals of the framework of the radiator system.

Thus compositions within the scope of the invention usually contain a monohydric aliphatic alcohol containing up to about six carbon atoms, a lower glycol, glycerol or a mixture thereof; water; the phthalate compound; an anti-leak agent such as linseed when a glycol is employed; sometimes an anti-foaming agent especially when a glycol is employed; and sometimes a dye material. In preparing compositions according to the invention a concentrated composition is first prepared and then by diluting the concentrate with water in various amounts the hydraulic

media of various freezing points are prepared. The amount of the phthalate added as a corrosion inhibitor varies between about 0.1% and 2.0% of the weight of the composition that is prepared as a concentrate.

An example illustrative of the invention has the following composition:

|                                                                      | Per cent  |
|----------------------------------------------------------------------|-----------|
| Mixture of methyl and isopropyl alcohols<br>(specific gravity 0.809) | 99        |
| Water                                                                | 1         |
| To which is added                                                    |           |
|                                                                      | Gms./gal. |
| Phthalate corrosion inhibitor                                        | 4         |
| Sodium nitrite                                                       | 8         |
| National Alphazurine-2G-dye                                          | 0.04      |

This composition is illustrative of a concentrate which is capable of dilution with water in any degree and thus permits the preparation of hydraulic media for a wide range of low temperature characteristics. Thus for protection to temperatures of about 20° F. a 15% aqueous solution is prepared and for temperatures of about 0° F. a 30% aqueous solution is prepared.

In the preparation of concentrates according to the above type, mixtures of methyl and isopropyl alcohols may vary in ranges from 90 to 10% of methyl alcohol and from 10 to 90% of isopropyl alcohol. Instead of such alcohols, ethyl alcohol or any of the other lower aliphatic monohydric, or dihydric alcohols or glycerol may be used. The alcohols which are suitable in this invention are the monohydric and polyhydric aliphatic alcohols containing up to six carbon atoms in the molecule, and of these the preferred alcohols are those containing one to four carbon atoms in the molecule, and particularly methyl, ethyl, propyl and isopropyl alcohols, ethylene glycol and 1-2 propylene glycol and glycerol. Advantages of using the glycols and glycerols are that in addition to their low freezing and high boiling points they become highly viscous at low temperatures before solidifying, and that except for the very dilute aqueous solutions expansion at low temperatures does not crack the radiator or engine block of the automobile.

A disadvantage of using certain of alcohol compounds especially the glycols in the preparation of anti-freeze solutions is that of imparting to the composition a capacity to leak and creep through minute solder pores and crevices. To counteract such losses of material compounds of the type of linseed meal are incorporated in the compositions. Other compounds which may be used to reduce leakage are gum gambier, tragacanth, quince seed, Irish moss and their mixtures. Other well dispersed solids may be included such as paper pulp, aluminum or bronze, but in general linseed or flax seed meal are preferred because of the superior results obtained and their clean appearance. The amounts in which these materials are incorporated in the anti-freeze composition are usually about 5 grams per gallon of concentrate.

The amount of water in the concentrated composition is roughly that given in the specific example, although less concentrated alcohols containing larger amounts of water may also be used.

The phthalates of the metals above aluminum in the specific example. These nitrites are added to the concentrated compositions in amounts between 0.5 and 8 grams per gallon and preferably in an amount between 2 and 5 grams per gallon. Of these phthalates the sodium com-

pound is generally used because of its low cost and its solubility in the alcohols.

The phthalate compounds employed in this invention have been found to give an added effect. Thus, the alkali metal nitrites have been employed in the prior art as anti-corrosive agents, but their use in anti-freeze solutions as corrosion inhibitors is disadvantageous because of their activity on solder in contact with copper. The phthalate compounds of this invention have the particularly desirable feature of repressing the corrosive activity of the alkali metal nitrites upon solder in contact with copper, while maintaining the advantageous effect of these nitrites in inhibiting the corrosion of iron. A composition containing both a phthalate and nitrite compound is exemplified in the specific concentrate shown as an embodiment of the invention.

The nitrite of any of the alkali metals may be employed instead of sodium nitrite as indicated in the specific example. These nitrates are added to the concentrates in amounts between 0.5 and 10 grams per gallon but usually the amount is between 1.5 and 6 grams per gallon.

The dye material is added in small amounts to the composition in order to impart distinctive and attractive appearance for sales purposes. Any suitable dye material can be used instead of National Alphazurine-2G as given in the specific composition which is presented as an illustration of the invention.

The order and method of mixing the various ingredients may be varied to suit the equipment available for blending. The blending equipment may be any suitable form of homogenizing means such as a colloid mill or equivalent device for producing violent agitation capable of effecting fine subdivision in the liquids of any materials that are likely to be suspended.

In order to demonstrate some of the favorable properties of the compositions tests were made on the following solutions:

|                                                                                                                                                                     | Per cent |
|---------------------------------------------------------------------------------------------------------------------------------------------------------------------|----------|
| Methyl alcohol                                                                                                                                                      | 66.0     |
| Iso propyl alcohol                                                                                                                                                  | 33.0     |
| Water                                                                                                                                                               | 1.0      |
| 75% (vol.) water                                                                                                                                                    |          |
| Tap water                                                                                                                                                           | 100      |
| 3. Composition as in (1) above, together with<br>Sodium nitrite, 8 gm./gal. of alcohol con-<br>centrate.                                                            |          |
| 4. Composition as in (1) above, together with<br>Sodium phthalate, 4 gm./gal. of alcohol<br>concentrate.                                                            |          |
| 5. Composition as in (1) above, together with<br>Sodium nitrite, 8 gm./gal. of alcohol con-<br>centrate.<br>Sodium phthalate, 4 gm./gal. of alcohol<br>concentrate. |          |

These compositions had freezing points below 10° F. It is correct to state that these compositions had freezing points of about 10° F. because at about that temperature super cooling and latent heat effects occur and throughout the mass the formation of small ice crystals is noticeable.

The above compositions were tested for corrosion by means of the following procedure:

Strips of various metals ( $\frac{1}{8}'' \times 3'' \times \frac{1}{4}''$ ) were fastened to a stainless steel support and immersed in the test solution to half their length in a suitable flask vented to the air by a long glass tube air condenser. The flask was placed in a constant temperature bath maintained at 71° C.  $\pm .5^{\circ}$  C. for 144 hours. The strips were carefully

cleaned and weighed before and after immersion. The total loss in weight expressed in milligrams represents the amount of corrosion. The lower the corrosion loss the more desirable the solution. Corrosion losses greater than 15 milligrams are considered objectionable degrees of corrosion.

The following results were obtained:

| Solution No.— | Weight differentials of strips |               |       |        |
|---------------|--------------------------------|---------------|-------|--------|
|               | Copper                         | Alumi-<br>num | Brass | Solder |
| 1.....        | -0.5                           | -1.8          | -0.3  | -1.7   |
| 2.....        | +1.0                           | -9.9          | +0.8  | +0.6   |
| 3.....        | +0.3                           | -3.6          | -0.6  | -11.8  |
| 4.....        | +0.4                           | +1.5          | +0.6  | +0.1   |
| 5.....        | +0.1                           | -8.0          | 0.0   | +0.8   |

These data indicate that the composition containing sodium phthalate has very low corrosive effects, especially upon solder and that the combination of sodium phthalate and sodium nitrite is particularly effective in suppressing corrosive tendencies of aqueous alcoholic solutions. Furthermore, it is reasonable to presume the rates of corrosion of the various metals under the conditions of the test are many times greater than those which would occur in the use of such liquids as cooling media in the automobile engine system. The above solutions containing sodium phthalate when tested in an automobile radiator did not develop foam or evaporate to an objectionable extent.

The description of the invention which has been given is illustrative. It is to be understood that while specific examples have been given for

purposes of illustration, the invention is not to be limited thereby. It is to be understood that the phthalate compounds disclosed in the description for incorporation in aqueous hydraulic media may be used either singly or in combination and that these phthalate compounds are as applicable to individual aliphatic alcohols of the range given as to mixtures thereof. Other means of applying the principle of the invention may be employed without departing from the scope of the invention so long as the ingredients stated by any of the following claims or the equivalent of such stated ingredients be employed.

What is claimed is:

1. A liquid composition suitable for use in heat exchange and pressure transmitting devices comprising a mixture of an aliphatic alcohol containing up to 6 carbon atoms in the molecule and water as the main ingredients and a quantity of a phthalate of a metal above aluminum in the electromotive series in corrosion-inhibiting proportions, which phthalate has no substituted components on the benzene ring.
2. A liquid composition according to claim 1 in which the phthalate is an alkali metal phthalate.
3. A non-corrosive liquid composition suitable for use in the cooling systems of automobile engines which comprises a mixture of methyl and isopropyl alcohols and water as major ingredients and an alkali metal phthalate and sodium nitrite as minor constituents in corrosion-inhibiting proportions, the phthalate having no substituted components on the benzene ring.

THEODORE R. DONLAN.